

Patented May 12, 1931

1,804,899

## UNITED STATES PATENT OFFICE

HERMANN VON FORSTER, OF NIEDERURSEL, NEAR FRANKFORT-ON-THE-MAIN, AND  
EMIL LAY, OF ESCHERSHEIM, NEAR FRANKFORT-ON-THE-MAIN, GERMANY, ASSIGN-  
ORS TO METALLGESELLSCHAFT AKTIENGESELLSCHAFT, OF FRANKFORT-ON-THE-  
MAIN, GERMANY, A CORPORATION OF GERMANY

### COMPOSITE METAL

No Drawing. Application filed September 11, 1929, Serial No. 391,982, and in Germany April 20, 1927.

This invention relates to composite metals, produced by welding coating metals on to iron cores, preferably by the casting-on process.

5 A great variety of coating metals have already been proposed for use in the production of composite metals. If, however, the composite metal is to be subjected to treatment, such as hot rolling, to produce a 10 change of shape, substantially the only composite metals that could be used for this purpose were those in which copper formed the coating metal. Coating metals consisting of copper alloys, such as brass, were 15 unsuitable, since in such case the hot shaping treatment rendered the workpiece useless although, in themselves, brass alloys and particularly such alloys as contain 55-60% of copper, can be worked by hot rolling. By maintaining suitable conditions, it 20 is also possible to hot roll and forge grades of brass with a still higher content of copper. A small addition of iron or manganese increases the workability of the material at 25 red heat, whereas even as little as 0.5% of lead impairs the suitability for rolling.

In hot rolling composite metals, however, the coating metal must comply with requirements which are entirely different from 30 those in cases where the coating metal is to be worked by itself. For instance, in the case of composite metals the coating metal must be able not only to stand the shaping treatment perfectly, but also there must be 35 no loosening of the welded union between it and the core metal. Since, in addition, the iron core is generally substantially harder than the brass alloy, the brass alloy would sustain an incomparably greater stress at 40 the weld surface, in rolling, than if worked separately. It was therefore impossible to ascertain in advance whether a brass alloy which could be satisfactorily hot rolled, could also be used as coating metal for a 45 composite metal to be hot rolled, and, as a matter of fact, it has been found that brass alloys containing less than 60% of copper (which, as is well known, are the most suitable for hot rolling) cannot be employed for 50 this purpose.

The present invention contemplates the production of a composite metal suitable for hot rolling, by welding copper-zinc alloys containing more than 60% of copper, as a coating, on to an iron core. It has been 55 found that bimetallic wire can be successfully made from rolled bars, produced by casting brass around iron ingots, provided the brass be made, not from the commercial 60 grades of zinc hitherto used, but from zinc containing less than 0.01% of lead. The total lead content of the alloy should not exceed 0.01%. In addition 0.05-1% of manganese may be incorporated in such brass.

Ingots of this kind can be rolled down 65 into wire by the usual process without difficulty. The capacity for rolling can be further improved by incorporating in the brass an amount of iron exceeding that which always dissolves in the coating metal in the casting-on process and which is adequate for a satisfactory welded union. The dissolving 70 of iron in the cast-on metal should rather proceed to such an extent as also to affect the texture of the cast-on metal. This result is advantageously attained by maintaining, for a certain time during the welding process or that of casting on to the iron core, a temperature which is favourable to 75 the dissolution of the iron in the cast-on metal, the time and temperature being determined by the amount of core metal it is desired to transfer into the coating metal. The iron may, of course, also be introduced 80 in other ways; nevertheless, the procedure set forth affords the particular advantage that the iron content in the brass coating, within certain limits progressively decreases 85 from the iron core outwards. In this manner the maximum fineness of grain is obtained at the place where the composite metal is subjected to the maximum stress 90 during hot rolling, whilst the outer zones, which have taken up the smallest amount 95 of iron, retain the original properties of the brass, such as colour, ductility, and the like.

The herein-described process enables products which are completely free from defects, and similar to those obtained in the 100

manufacture of iron and copper wires to be produced.

We claim:

- 5 1. A composite metal produced by welding a coating of copper-zinc alloy onto an iron core by the casting-on process, characterized in that the copper-zinc alloy contains over 60% of copper and less than 0.01% of lead.
  - 10 2. Composite metal as set forth in claim 1 in which 0.05-1% of manganese is alloyed with the copper-zinc alloy.
  - 15 3. Composite metal as set forth in claim 1, in which copper-zinc alloy contains a small proportion of iron.
  - 20 4. Composite metal as set forth in claim 1, in which the copper-zinc alloy contains 0.05-1% of manganese and a small amount of iron.
- 20 In testimony whereof we affix our signatures.

HERMANN v. FORSTER.  
Dr. EMIL LAY.

25

30

35

40

45

50

55

60

65